

# United States Patent Office

3,810,837

1

3.810.837

3,810,637  
**OVERBASED SULFURIZED CALCIUM  
ALKYLPHENOLATE MANUFACTURE**

**AKER-CHAFETZ MANUFACTURE**  
Harry Chafetz, Poughkeepsie, William H. Channing,  
Wappingers Falls, and Bertrand G. Morissette, Beacon,  
N.Y., assignors to Texaco Inc., New York, N.Y.

No Drawing. Filed June 27, 1972. Ser. No. 366,836.

Int. Cl. C10m 1/54

U.S. Cl. 252—42 F 5 Claims

J. M. COOK 1754

## 5 Claims

## ABSTRACT OF THE DISCLOSURE

A method of preparing overbased sulfurized alkylphenolate of antioxidant properties in hydrocarbon lubricating oil comprising first heating a mixture of sulfurized normal calcium alkylphenolate, calcium oxide, alkanoic acid of from 2 to 3 carbons, alkoxyethanol of the formula  $\text{ROCH}_2\text{CH}_2\text{OH}$  where R is alkyl of from 1 to 4 carbons, and lubricating oil and subsequently contacting the heated mixture with carbon dioxide.

## BACKGROUND OF INVENTION

### Field of invention

This invention is in the field of art relating to fluent compositions specialized and designed for the use of between two relatively moving surfaces in contact therewith for reducing friction therebetween and preserving the surface. The lubricant compositions produced by the method of the invention contain a compound which has a calcium component linked to a carbon through an oxygen.

### Prior art

It is well known that lubricating oils tend to deteriorate under the conditions of use in present day diesel and automotive engines with attendant formations of sludge and lacquer and resinous materials which adhere to the engine parts, particularly the piston rings, grooves and skirt thereby lowering the operating efficiency of the engine. To counteract the formation of these deposits, certain chemical additives have been found which when added to lubricating oils have the ability to keep the deposit forming materials suspended in oil so that the engine is kept clean and in an efficient operation condition for extended periods of time. These agents are known in the art as detergents or dispersants. Metal organic compounds are particularly useful in this respect. These metal organic compounds are considered to be effective because they provide alkalinity to neutralize strong organic and inorganic acids and are capable of dispersing deposits and deposit precursors in the oil phase. Over-based sulfurized metal alkylphenolates have been found to be particularly effective dispersants in lubricating oils.

Heretofore and hereinafter by the term "overbased" it is meant that the ratio of the number of equivalents of calcium moiety to the number of equivalents of phenol moiety is greater than one, i.e., the calcium metal ratio is greater than one. In contrast, the equivalent ratio of calcium moiety to phenol moiety in sulfurized normal calcium alkylphenolate is 1:1, i.e., a calcium metal ratio of 1.

The prior art teaches many methods of preparing overbased sulfurized alkylphenolates. In one prior procedure the manufacture of lubricating oil compositions containing overbased sulfurized calcium alkylphenolate comprises introducing  $\text{CO}_2$  into a mixture of lubricating oil, a sulfurized normal calcium alkylphenolate at an elevated temperature, reacting the resultant mixture with ethylene glycol and calcium hydroxide to form the overbased salt. The sulfurized normal calcium alkylphenolate reactant

1

is manufactured therein by heating together a mixture of lubricating oil, alkylphenol, calcium hydroxide, elemental sulfur and a glycol.

Another prior procedure calls for introducing CO<sub>2</sub> into a mixture of lubricating oil, sulfurized normal calcium alkylphenolate, ethylene glycol or propylene glycol, calcium oxide or calcium hydroxide, a higher alkanol of 8 to 18 carbons and a dispersant, namely, an overbased alkaline earth metal hydrocarbon sulfonate.

10 Although these two methods produce satisfactory over-  
based sulfurized calcium alkylphenolates, they do have the  
disadvantage of requiring the use of ethylene glycol which  
is difficult to remove from the final reaction mixture. The  
presence of residual glycol in the final product is undesir-  
15 able since it tends to degrade the high temperature dis-  
persant properties of the product. Further, in respect to  
one prior method, a sulfonate dispersant is required in the  
initial reaction mixture and the presence of this sulfonate  
in the reaction mixture undesirably adds to the cost and  
20 undesirably excludes the final product from all uses where-  
in a sulfonate dispersant is prohibited since the sulfonate  
dispersant will be carried over into the final product and  
is not readily subject to separation.

To overcome the foregoing deficiencies, another prior method called for sequentially contacting a sulfurized normal calcium alkylphenolate with a calcium alkoxy-alkoxide such as calcium methoxyethoxide, preferably in the presence of an alkoxyalkanol, and then hydrolyzing between about 20 and 70 wt. percent of the overbased product. Although this latter method obviates the use of unattractive glycol, it does have the undesirable feature of consuming relatively expensive calcium 2-alkoxyalkoxide which is not recoverable.

## SUMMARY OF INVENTION

The subject invention relates to a novel method of producing overbased sulfurized calcium alkylphenolate containing lube oil compositions employing low cost over-basing ingredients, namely, calcium oxide and carbon dioxide and further utilizing a recoverable non-glycol reaction accelerator solvent medium combination of alkoxy-alkanol and lower alkanoic acid. More specifically, the method of the invention comprises heating in a lubricating oil medium a mixture of normal sulfurized calcium alkylphenolate, calcium oxide, alkanoic acid, alkoxy-alkanol and subsequently contacting the heated mixture with carbon dioxide.

## DETAILED DESCRIPTION OF THE INVENTION

In more detail, the method of the invention comprises heating a mixture of a sulfurized normal calcium alkyl-phenolate usually having a sulfur content between about 0.5 and 12 wt. percent, a calcium content between about 1 and 8 wt. percent and a total base number between about 55 and 225 which is characterized by the theoretical formula:



70 calcium oxide, alkanoic acid of from 2 to 3 carbons, alkoxyethanol of the formula  $\text{ROCH}_2\text{CH}_2\text{OH}$ , and hydrocarbon lubricating oil medium and subsequently contact-

ing the heated mixture with carbon dioxide to form a lube oil composition containing sulfurized calcium alkylphenolate characterized by the theoretical formula



where  $Q$  represents said sulfurized normal calcium alkylphenolate,  $R^1$  is a monovalent saturated aliphatic hydrocarbon radical (alkyl) from 4 to 100 carbons,  $x$  is an average integer of from 1 to 4,  $y$  is an average integer of from 0 to 10,  $R$  is alkyl of from 1 to 4 carbons and  $n$  is an average integer of 0.1 to 2 and higher. It is to be noted when  $n$  is 0.1 the overbased product is represented as having a calcium metal ratio of 1.1 and when  $n$  is 1 the calcium metal ratio is 2. The sulfur content of the overbased product is normally between about 0.5 and 12 wt. percent, the calcium content is between about 3.5 and 12 wt. percent and the calcium metal ratio is between about 1.5 and 2.5.

It is to be noted that  $x$  and  $y$  in the foregoing formulas defining the sulfurized calcium alkylphenolate are defined as average integers since sulfurized normal and sulfurized overbased calcium alkylphenolates in essence are a complex mixture of monosulfide and polysulfide or a mixture of polysulfide as theoretically defined. In any case, the  $R'$  group is mainly in the para position with the sulfur links mainly in the ortho position. Further, there is probably also a significant amount of covalent character to the calcium-oxygen bond.

During the  $CO_2$  contact the  $CO_2$  gas is introduced directly into the heated mixture, preferably by blowing therethrough. The heating of the mixture is advantageously conducted at a temperature between about 100 and 250° C., preferably between 150 and 200° C., and the  $CO_2$  contacting is conducted at a temperature of between about 100 and 250° C., preferably between about 150 and 225° C. In respect to ingredient quantities, a mole ratio of calcium oxide to sulfurized normal calcium alkylphenolate is desirably between about 1:1 and 3:1, preferably between 1:1 and 1.5:1, the mole ratio of calcium oxide to acetic acid is between about 2:1 and 30:1, preferably between 2.5:1 and 12:1, the mole ratio of calcium oxide to alkoxyalkanol is between about .02:1 and 0.3:1, preferably between .04:1 and 0.2:1 and the mole ratio of  $CO_2$  to calcium oxide is at least about 1:1 and up to 4:1 and higher, preferably between about 1:1 and 1.5:1. The lubricating oil medium can constitute between about 10 and 90 wt. percent of the reaction mixture, desirably between about 30 and 70 wt. percent resulting in a final lubricating oil medium can constitute between about 10 based calcium salt concentrate of between about 10 and 90 wt. percent, preferably between about 30 and 70 wt. percent.

Under advantageous conditions, the heated reaction mixture prior to  $CO_2$  contact is heated to a temperature within the contemplated temperature under reduced pressure, if necessary, to insure the removal of the alkoxyethanol ingredient as overhead. Further, under advantageous conditions, an inert gas such as nitrogen is passed through the reaction mixture during the heating stage and also advantageously after  $CO_2$  contact. The inert gas rate is suitably between about 1 and 10 volume gas/volume liquid mixture/hour. Further, the heating stage is normally conducted for a period of between about 1 and 5 hours and the  $CO_2$  contact stage between about 1 and 3 hours.

The crude product may be purified by standard means such as by blowing the final product with inert gas to remove volatile by-products and unreacted reactants and filtering the blown mixture through a standard pressure filter plate at about 20 to 200° C. under about 0.1 and 100 p.s.i. pressure utilizing a diatomaceous earth filter aid.

Under preferred conditions, the reaction mixture is maintained in an agitated state to facilitate ingredient contact. Usually, such state is maintained by the passage of carbon dioxide and inert gas therethrough but if need

be stirring may be instituted for supplemental agitation.

In the method of the invention there are several material aspects:

In the first place, it is essential that both the alkanoic acid and alkoxyalkanol in addition to the other method ingredients as defined be employed otherwise essentially no overbasing occurs. Further, the aforementioned temperature ranges and quantity ranges are required in order to obtain satisfactory overbasing in the desired range.

As heretofore indicated the products of the claimed method are lube oil concentrates of the overbased sulfurized calcium alkylphenolate wherein the overbased alkylphenolate content is between about 10 and 90 wt. percent. In finished lubricating oil compositions ready for automotive use, the overbased additive content is advantageously between about 0.1 and 10 wt. percent, and therefore, the final product is normally subject to additional dilution with hydrocarbon lubricating oil before use. In the finished lubricating oil compositions suitable for use in automotive engines, additives in addition to the overbased sulfurized calcium alkylphenolates may be included. These other additives may be any of the standard suitable pour depressors, additional sludge dispersants (e.g., petroleum sulfonates), antioxidants, silver corrosion inhibitors, viscosity index improvers and oiliness agents. Exactly what other additives are included in the finished oil and the particular amounts thereof will, of course, depend on the particular use and conditions desired for the finished oil product.

Suitable base oils useful in the manufacture of the overbased phenolates include a wide variety of hydrocarbon lubricating oils such as naphthenic base, paraffinic base and mixed base mineral oils of other hydrocarbon lubricants, e.g., lubricating oils derived from coal products and synthetic oils, e.g., alkylene polymers such as polypropylene and polyisobutylene of a molecular weight between about 250 and 2500. Advantageously, lubricating base oils having an SUS viscosity at 100° F. between about 50 and 2000, preferably between about 100 and 300 are employed.

Examples of the sulfurized calcium alkylphenolate reactants based on the theoretical formula:



are where  $R'$  is 4-octyl,  $x$  is 1 and  $y$  is 0;  $R'$  is 4-dodecyl,  $x$  is 1 and  $y$  is 1;  $R'$  is 4-eicosyl,  $x$  is 2 and  $y$  is 2;  $R'$  is 4-dodecyl,  $x$  is 2 and  $y$  is 3; and mixtures thereof. It is to be noted that  $x$  and  $y$  are defined as average integers. Further description and method of preparing sulfurized normal calcium alkylphenolates are set forth in U.S. 3,528,971 and 3,549,534. Briefly, the normal salt reactants are prepared by reacting an alkylphenol characterized by the formula



with a calcium compound such as calcium alkoxyalkoxide, e.g., calcium-2-methoxyethoxide followed by reacting the resultant reaction product with sulfur. Examples of the alkylphenol precursors contemplated herein are 4-octylphenol, 4-t-octylphenol, 2-decylphenol, 2-dodecylphenol, 4-hexadecylphenol, 2,4-didodecylphenol, 2-nonylphenol, 4-tricosylphenol, 4-eicosylphenol, a mixture of decylphenol and dodecylphenol ( $C_{10} + C_{12}$  alkylphenol) and mixtures of 2 and 4 positioned monoalkyl and dialkylphenol. The only restriction is at least one ortho or para position be available for sulfurization.

Examples of the alkoxyalkanols contemplated herein are 2-methoxyethanol, 2-ethoxyethanol, 2-propoxyethanol, 2-isopropoxyethanol and 2-butoxyethanol.

Specific examples of the alkanoic acids contemplated herein are acetic acid and propanoic acid.

The following examples illustrate the method of the invention but are not to be construed as limitations thereof.

#### Example I

This example illustrates the method of the invention.

A mixture of 13 grams (0.23 mole) of calcium oxide, 1.2 grams (0.02 mole) of acetic acid and 500 mls. (6.4 moles) of 2-methoxyethanol were refluxed (128° C.) for a period of 3 hours during which time nitrogen gas was continually passed therethrough at a rate of 50 mls./minute. To the resultant refluxed mixture there were added 20 grams of naphthenic lubricating oil having an SUS viscosity of about 100 at 100° F. and 270 grams (approx. 0.2 mole) of a 50 wt. percent lube oil solution of sulfurized normal calcium-4-C<sub>10</sub>+C<sub>12</sub> alkylphenolate of a calcium ratio of 1, the lube oil solution having a calcium content of 2.85 wt. percent, a sulfur content of 3.3 wt. percent, a total base number of 80, the lube oil component being a naphthenic lubricating oil having an SUS viscosity of about 100 at 100° F. The resultant mixture was heated and stripped to 210° C. with the heating continued at this temperature for a period of 2 hours. Nitrogen gas was passed through the reaction mixture at a rate of 50 mls./minute. At the end of the 2 hour period the nitrogen blowing was ceased and carbon dioxide was passed through the reaction mixture at a rate of 100 mls./minute for a period of 1 hour at a temperature of 210° C. representing an introduction of approximately 0.27 mole CO<sub>2</sub>. At the end of the 2 hour period, the resultant mixture was finally blown with nitrogen at a rate of 50 mls./minute for a period of 1 hour at 210° C. and the blown mixture was filtered through diatomaceous earth at 150° C. The filtered product was found to be a 50 wt. percent lubricating oil solution of overbased sulfurized calcium alkylphenolate having a metal ratio of 2.0, the filtered product having a calcium content of 5.1 wt. percent (5.4 calcd.), a total base number of 139 (151 calcd.) and a sulfur content of 2.8 wt. percent.

#### Example II

This example further illustrates the method of the invention.

A mixture was prepared consisting of 14 grams (0.25 mole) of calcium oxide, 6 grams (0.1 mole) of acetic acid, 20 grams of naphthenic lubricating oil of an SUS viscosity of about 100 at 100° F., 200 mls. (2.5 moles) of 2-methoxyethanol and 270 grams (approx. 0.2 mole) of a 50 wt. percent lube oil solution of sulfurized normal calcium-4-C<sub>10</sub>+C<sub>12</sub> alkylphenolate of a calcium metal ratio of 1, said lube solution having a calcium content of 2.85 wt. percent, a sulfur content of 3.3 wt. percent, a total base number of 80, the oil component being naphthenic oil of an SUS viscosity of 100 at 100° F. The mixture was refluxed for 3 hours at 128° C. while passing nitrogen gas therethrough at a rate of 50 mls./minute. At the end of the 3 hour period, the reaction mixture was heated to 210° C. with the continued nitrogen blowing to strip off 2-methoxyethanol and the 210° C. temperature was maintained for a 4 hour period. At the end of the 4 hour period the nitrogen blowing was ceased and carbon dioxide was passed through the mixture for 1 hour at a rate of 100 mls./minute for a total introduction of 0.27 mole followed by nitrogen blowing at the previous nitrogen rate for 0.5 hour while maintaining the temperature at 210° C. The resultant product was filtered through diatomaceous earth and the clarified filtrate was determined to be a 50 wt. percent lube oil solution of overbased sulfurized calcium-4-C<sub>10</sub>+C<sub>12</sub> alkylphenolate of a

calcium metal ratio of 2.1, the solution having a calcium content of 5.3 wt. percent (5.7 wt. percent calcd.), a sulfur content of 2.8 wt. percent and a total base number of 141 (159 calcd.).

#### Example III

This example illustrates that overbasing will essentially not occur in the absence of the alkanoic acid ingredient.

There was formed a mixture of 21 grams (0.37 mole) of calcium oxide, 18 mls. (1.0 mole) of water, 100 mls. (1.3 moles) of 2-methoxyethanol, 22 grams of naphthenic lubricating oil of an SUS viscosity of about 100 at 100° F., and 200 grams (0.15 mole) of a 50 wt. percent lube oil solution containing normal sulfurized calcium-4-C<sub>10</sub>+C<sub>12</sub> alkylphenolate of a calcium metal ratio of 1, said solution having a calcium content of 2.95 wt. percent, a sulfur content of 2.7 wt. percent, the oil component being a naphthenic oil of an SUS viscosity of 100 at 100° F. The mixture was nitrogen stripped and CO<sub>2</sub> blown as in Example II and the resultant mixture was further stripped with nitrogen at a nitrogen rate of 50 mls./minute to a temperature of 180° C. and held for an additional 3 hours at this temperature. The product was filtered through diatomaceous earth and was found to be 50 wt. percent lube oil solution of the initial sulfurized normal calcium-4-C<sub>10</sub>+C<sub>12</sub> alkylphenolate of a calcium metal ratio of 1, said solution having a calcium content of 3 wt. percent, thereby demonstrating only minimal overbasing occurred.

#### Example IV

This example further illustrates that essentially no overbasing occurs in the absence of the alkanoic acid ingredient.

A mixture was formed consisting of 14 grams (0.25 mole) of calcium oxide, 200 mls. (2.5 moles) of 2-methoxyethanol, 20 grams naphthenic lubricating oil of an SUS viscosity of about 100 at 100° F., and 270 grams (about 0.2 mole) of a 50 wt. percent lube oil solution of sulfurized normal calcium-4-C<sub>10</sub>+C<sub>12</sub> alkylphenolate of a calcium metal ratio of 1, said solution having a calcium content of 3 wt. percent, a sulfur content of 2.9 wt. percent, a total base number of 86, the lube oil component being naphthenic oil of an SUS viscosity of about 100 at 100° F. The mixture was refluxed for a period of 3 hours at 127° C. while passing nitrogen gas therethrough at a rate of 50 mls./minute. It was then heated to 210° C. with continuous nitrogen blowing with stripping off the 2-methoxyethanol. It was held at 210° C. for a period of 4 hours. At the end of the 4 hour period and at 210° C. there was passed through the mixture for 1 hour 100 mls./minute of CO<sub>2</sub> or a total of 0.27 mole CO<sub>2</sub> followed by nitrogen blowing at the previous nitrogen rate for a 0.5 hour period while keeping the temperature at 210° C. The product was filtered through diatomaceous earth. The clarified product upon analysis was found to be a 50 wt. percent lube oil solution of essentially sulfurized normal calcium-4-C<sub>10</sub>+C<sub>12</sub> alkylphenolate, said phenolate having a calcium metal ratio of about 1.2, said solution having a calcium content of 3.4 wt. percent (5.7 wt. percent calcd.), a sulfur content of 3 wt. percent and a total base number of 96 (159 calcd.), thereby demonstrating that only minimal overbasing occurred.

#### Example V

This example illustrates the failure of satisfactory overbased product formation with the substitution of the alkoxyethanol ingredient with closely related ethylene glycol.

There was formed a mixture of 14 grams (0.25 mole) of calcium oxide, 6 grams (0.1 mole) of acetic acid, 20 grams of naphthenic lubricating oil of an SUS viscosity of 100 at 100° F., 200 mls. (3.6 moles) ethylene glycol, and 270 grams of a 50 wt. percent lube oil solu-

tion of sulfurized normal calcium alkylphenolate of a calcium metal ratio of about 1, said solution having a calcium content of 2.90 wt. percent, a sulfur content of 3.0 wt. percent and a total base number of 80, the lube component being naphthenic lube oil of an SUS viscosity at 100° F. of 100. The resultant mixture was heated for 3 hours at 150° C. while passing a nitrogen therethrough at a rate of 50 mls./minute. At the end of the 3 hour period, carbon dioxide was then passed through the mixture for 1 hour at a rate of 100 mls./minute representing a total carbon dioxide introduction of 0.27 mole and then nitrogen was introduced for a period of 1 hour at a rate of 50 mls./minute while maintaining the temperature at 150° C. At the end of the 1 hour period the reaction mixture was heated to 210° C. under a reduced pressure of 15 mm. Hg while removing ethylene glycol as overhead and held at this temperature for a 1 hour period. The product was filtered through diatomaceous earth. The product was unstable in that significant quantities of calcium containing solids continually settled out of it. The foregoing indicates that a stable overbased sulfurized calcium alkylphenolate could not be made when ethylene glycol was substituted for the alkoxyalkanol under the foregoing conditions. Such settling did not occur in Examples I and II representing the procedure of the invention.

#### Example VI

This example illustrates the failure of overbasing to take place in the absence of the alkoxyethanol ingredient.

There was formed a mixture of 13 grams (0.23 mole) of calcium oxide, 6 grams (0.1 mole) of acetic acid, 20 grams of naphthenic lubricating oil of an SUS viscosity of 100 at 100° F. and 260 grams (0.2 mole) of a 50 wt. percent lube oil solution of sulfurized normal calcium alkylphenolate of a calcium metal ratio of about 1; said solution having a calcium content of 3.0 wt. percent, a sulfur content of 3.3 wt. percent and a total base number of 80, the lube component being naphthenic lube oil of an SUS viscosity of 100° F. of 100. The resultant mixture was heated for 4 hours at 204° C. while passing a nitrogen therethrough at a rate of 50 mls./minute. At the end of the 4 hour period, carbon dioxide was passed through the mixture for 1 hour at a rate of 100 mls./minute representing a total carbon dioxide introduction of 0.27 mole and then nitrogen was introduced for a period of 0.5 hour at a rate of 50 mls./minute while maintaining the temperature at 210° C. The product was filtered through diatomaceous earth and the filtrate analyzed. It was determined to be a 50 wt. percent lube oil solution of sulfurized normal calcium-4-C<sub>10</sub>+C<sub>12</sub> alkylphenolate, said alkylphenolate per se having a calcium metal ratio of 1, the solution having a calcium content of 2.8 wt. percent and a sulfur content of 3.1 wt. percent and a total base number of 78. The foregoing indicates that essentially no overbasing took place.

We claim:

1. A method of preparing a lubricating oil composition containing an overbased sulfurized calcium alkylphenolate wherein said alkyl group is of from 4 to 100 carbons consisting essentially of first heating a mixture of calcium oxide, an alkanoic acid selected from acetic acid or propanoic acid, alkoxyethanol of the formula ROCH<sub>2</sub>CH<sub>2</sub>OH where R is alkyl of from 1 to 4 carbons, a hydrocarbon lubricating oil of an SUS viscosity at 100° F. of between about 50 and 2000 and a sulfurized normal calcium alkylphenolate wherein said alkyl is as heretofore defined, at a first temperature of between about 100 and 250° C., subsequently introducing into the reaction mixture carbon dioxide in a total amount of at least about 1 mole per mole of said calcium oxide, at a second temperature between about 100 and 250° C. and recovering said lubricating oil composition, in said mixture, said lubricating oil being present in a major amount, the initial mole ratio in said mixture of calcium oxide to acetic acid being between about 2:1 and 30:1, the initial mole ratio in said mixture of calcium oxide to said normal sulfurized calcium alkylphenolate being between about 1:1 and 3:1, the initial mole ratio of calcium oxide to alkoxyalkanol being between about .02:1 and 0.3:1.

2. A method in accordance with claim 1 wherein said acid is acetic acid and said alkoxyethanol is 2-methoxyethanol.

3. A method in accordance with claim 1 wherein in said first heating and subsequent to said CO<sub>2</sub> introduction an inert gas is passed through the reaction mixture at a rate of between about 1 to 10 vol. gas/vol. reaction mixture/hour.

4. A method in accordance with claim 1 wherein in said first heating said calcium oxide, said alkanoic acid and said alkoxyethanol is first heated at said first temperature followed by the subsequent introduction of said hydrocarbon lubricating oil and said sulfurized normal calcium alkylphenolate followed by the removal of said alkoxyalkanol as overhead.

5. A method in accordance with claim 4 wherein said alkanoic acid is acetic acid and said alkoxyethanol is 2-methoxyethanol.

#### References Cited

##### UNITED STATES PATENTS

|           |         |                |       |          |
|-----------|---------|----------------|-------|----------|
| 3,350,310 | 10/1967 | Herd et al.    | ----- | 252—42.7 |
| 3,493,516 | 2/1970  | Allphin et al. | ----- | 252—18 X |
| 3,544,463 | 12/1970 | Koft           | ----- | 252—40.7 |

PATRICK P. GARVIN, Primary Examiner

A. H. METZ, Assistant Examiner

U.S. CL. X.R.

252—18, 40.7